

## UNITED STATES PATENT OFFICE

2,141,110

## TIN PLATE

Charles E. Miller, Gary, Ind.

No Drawing. Application November 24, 1936,  
Serial No. 112,609

## 2 Claims. (Cl. 91—70.3)

This invention relates to tin plate, one of the objects being to produce this product so that it will successfully meet the hydrogen-evolution tests used by customers to test its corrosion resistance, regardless of the location of the portion of its surface to which this test is applied.

It is to be understood that tin plate consists of steel coated with tin, and that this steel may be produced by either the hot-rolling or cold-rolling methods. This invention is particularly concerned with cold-rolled tin plate and is characterized by the step of conditioning the surface of the cold-rolled steel so that when it is passed through the tinning machines its surface carries sufficient tin into the tinning rolls to permit the latter to more uniformly distribute the tin over the length of the steel.

An example of this conditioning is to slightly roughen the surface of the cold-rolled steel, which is normally denser and smoother than the surface of the hot-rolled steel. This roughening may be done by passing the steel through cold-rolls that are slightly rougher than are used for cold-rolling purposes, the roughness of the rolls being such that the surface of the cold-rolled steel is rougher when it leaves these rolls than cold-rolled steel but is not so rough as hot-rolled steel. The cold-working rolls may be roughened for this purpose by grinding them with an abrasive wheel of the proper grit number; also, the rolls may be shot-blasted.

The described roughening of the cold-rolled steel may be done during the temper-rolling required to adjust the stiffness of such steel subsequent to its being annealed to remove the severe hardness induced by the cold-rolling which brought it to gage. The other processing required in the production of the tin plate may be conventional. That is to say, after the steel is roughened it may be cleansed and passed through a conventional tinning machine where it is fluxed, dipped into molten tin and passed through tinning rolls which adjust and distribute the tin over its surface.

Some experimentation may be necessary to determine the degree of roughening to which the steel must be subjected, in view of variations in tinning practice. However, once the funda-

mental principle is understood the practice of the invention is an easy matter. If the steel is not roughened sufficiently prior to tinning it will be found that insufficient tin is carried by the trailing portion of the plate which, incidentally, is 5 contrary to the troubles encountered in tinning hot-rolled steel when the plate is inclined to carry too much tin on this portion. If the surface of the cold-rolled steel is roughened too much the same trouble will be experienced as is involved by 10 the use of hot-rolled steel. It follows that it is obviously possible to determine when the proper degree of roughness has been imparted to the steel, since the tin will be applied by the tinning machine with substantial uniformity from end- 15 to-end or lengthwise of the sheet.

The product resulting from this method possesses greater corrosion resistance than tin plate produced according to the prior art regardless of whether the steel is hot or cold-rolled. As just mentioned, it is impossible to secure uniform distribution of the tin in both instances. However, the plate produced according to the present invention may be made to carry its tin with substantial uniformity over its entire surface area, 25 whereby for a given weight of tin greater corrosion protection is secured.

## I claim:

1. A method of producing tin plate from cold rolled steel, including rendering the surface of said steel rougher than normal but not so rough as the normal surface of hot rolled steel and subsequently passing said steel through a tinning machine.

2. A method of producing tin plate from cold rolled steel, including passing said steel through a tinning machine and roughening the surface of said steel prior to passing through said machine to a sufficient degree to cause it to carry sufficient tin into the tinning rolls of said machine to permit the same to adjust the tin so the coating on the leading parts of said surface is not substantially greater in thickness than it is on the following parts, said roughening being insufficient to cause said rolls to adjust said coating so it is thicker on the trailing parts of said steel than it is on said leading parts.

CHARLES E. MILLER.